

## 1

2,816,870

## DISPERSLBLE FATTY AMINES

Thomas H. Lentz, St. Louis Park, and Joseph W. Opie and David E. Terry, Minneapolis, Minn., assignors to General Mills, Inc., a corporation of Delaware

No Drawing. Application July 19, 1954,  
Serial No. 444,355

5 Claims. (Cl. 252—61)

The present invention relates to a composition composed largely of higher fatty amines in such a form that they are readily dispersible in water.

The higher fatty amines, especially those derived from tallow fatty acids, are used in very large quantities in mineral flotation operations. To obtain the maximum results from a fatty collector, such as tallow amine, the amine must be thoroughly dispersed in the aqueous phase of a flotation pulp. It is then completely available to acidic minerals such as silica for surface adsorption and subsequent flotation. Since only a mono-molecular layer of collector is necessary to float sized mineral particles, and only 5% surface coating renders a mineral particle floatable, complete dispersion of collector prior to the attachment to a mineral surface facilitates the adsorption of single molecules rather than several molecular layers. Consequently the amine collector can be used in a most efficacious manner and in smaller quantities in a dispersed form than can chemically identical non-dispersible amines.

It is, therefore, an object of the present invention to provide a novel fatty amine composition which is readily dispersible in water.

The invention is applicable to the long chain fatty amines in general. It is particularly adapted to the longer chain amines such as those containing 14-22 or more carbon atoms. These amines are frequently solid or soft semi-solid materials which are very viscous and, accordingly, are very difficult to disperse. The tallow amines are used very extensively for commercial flotation. Tallow amines in general are composed of a mixture of amines comprising approximately 50% oleylamine and approximately 50% a mixture of palmityl and stearylamine. It is evident that amines for flotation may be made from the fatty acids of other fats or oils, both animal and vegetable. The amines may be isolated pure amines but in general would be a mixture of the amines from the whole fat or oil or from some selected fraction thereof. The amines may be either saturated or unsaturated or mixtures thereof.

The composition of the present invention is composed of the long chain fatty amine, a solvent therefor in the form of an alkoxyalkanol and a dispersing agent. The alkoxyalkanol suitable for the present invention has the following formula:



in which R is an alkyl group containing from 1-4 carbon atoms. Typical compounds suitable for this purpose are 2-ethoxyethanol, butoxyethanol, 2-methoxyethanol and the like.

## 2

The dispersing agent may be either a cationic or a nonionic dispersing agent. Any compound in this category may be used for this purpose. Typical dispersing agents include polyoxyethylene esters of mixed fatty and 5 rosin acids and substituted oxazolines. In view of the cationic nature of the amine it is possible to prepare a dispersing agent by simply neutralizing a small portion of the amine with a suitable acid such as acetic acid. When from 2-3% of the amines are neutralized the intrinsic 10 emulsifying agent formed was found to give excellent emulsification of the composition.

It is preferred to include as high a concentration of the amines in the composition as possible, while still obtaining a readily dispersible and fluid product. Generally it is not necessary to use sufficient of the solvent 15 to dissolve completely all of the amine. Sufficient solvent is employed to render the composition fluid and dispersible. Generally the preferred compositions contain sufficient solvent so that 75-95% of the amine is dissolved and from 5-25% of the amine by weight may be in the form of suspended solids. Usually from 10-20% of the solvent is sufficient to accomplish this result. The remaining 80-90% of the composition is the fatty amine containing only a small quantity of dispersant. For example a typical composition is one composed of approximately 85% technical grade tallow amines, 15% of 2-ethoxy ethanol and a small quantity of acetic acid sufficient to neutralize from 2-3% of the amine. In this 20 composition from 10-15% by weight of the amines remain undissolved but the composition is fluid and is readily dispersible in water. In place of acetic acid for neutralization of the amine any acid which is sufficiently reactive to form an amine salt may be used. Typical 25 acids include formic, glycolic, hydrochloric, and the like.

## EXAMPLE 1

Technical tallow amine and 2-ethoxyethanol and acetic acid were blended together in the proportions indicated in the following table. The compositions obtained were 30 fluid at room temperature and contained the indicated quantities of undispersed solids notwithstanding the presence of the undispersed solids the materials were fluid and were readily dispersible in water. Samples of these 35 materials were dispersed in cold tap water to produce a 5% dispersion. The stability of these dispersions is likewise disclosed in the following table. This shows that even a minute quantity of acetic acid serves to effect some dispersibility of the composition but that the optimum quantity of acetic acid appears to be approximately 0.5% which is approximately enough to form the 40 amine salts of about 2-3% of the tallow amine.

| 55     | Sample | Techni-<br>cal<br>Tallow<br>Amine | 2-ethoxy-<br>ethanol | Acetic<br>Acid | Percent<br>Solids at<br>Room<br>Temp. | 5% Disper-<br>sion in Cold<br>Tap Water |
|--------|--------|-----------------------------------|----------------------|----------------|---------------------------------------|-----------------------------------------|
| 1----- |        | 85                                | 14.9                 | 0.1            | 10                                    | Breaks after<br>1 hr.                   |
| 2----- |        | 85                                | 14.5                 | 0.5            | 13                                    | Stable.                                 |
| 3----- |        | 85                                | 14                   | 1.0            | 15                                    | Do.                                     |

## EXAMPLE 2

Composition No. 2 from Example 1 was used for the 65 flotation of silica from phosphate rock. A similar flotation was performed employing the acetate of technical tal-

low amine as a flotation agent. This technical tallow amine acetate is a conventional flotation agent. The results are indicated in the following table:

*Phosphate beneficiation with fluid tallow amines*

|                                                                              | lbs.<br>re-<br>agent<br>per<br>ton | Phosphate Concentrate |                |              |                          | Silica Tailing |                |              |                            |
|------------------------------------------------------------------------------|------------------------------------|-----------------------|----------------|--------------|--------------------------|----------------|----------------|--------------|----------------------------|
|                                                                              |                                    | Percent<br>Wt.        | Percent<br>BPL | BPL<br>Units | Percent<br>HCl<br>Insol. | Percent<br>Wt. | Percent<br>BPL | BPL<br>Units | Percent<br>BPL<br>Recovery |
| 1. 85% Technical Tallow<br>Amine, 14½% 2-ethoxy-<br>ethanol, ½% Acetic Acid. | 0.32                               | 90.0                  | 81.1           | 73.0         | 3.63                     | 10.0           | 12.4           | 1.2          | 98.6                       |
| 2. Acetate of Technical Tallow<br>Amine.....                                 | 0.36                               | 89.4                  | 82.0           | 73.3         | 4.52                     | 10.6           | 6.3            | 0.7          | 99.1                       |

This table shows that approximately equivalent results were obtained in the two instances notwithstanding the fact that where the amine had been fluidized approximately 10% less amine was used. A saving in amine is thereby obtained in addition to the ease of obtaining dispersion of the amine product.

**EXAMPLE 3**

A reagent was prepared from 80% of technical tallow amine, 19½% of 2-ethoxy ethanol and 0.5% acetic acid. The reagent was fluid and contained approximately 5% solids by weight. It dispersed in water readily to produce a 5% stable dispersion.

This reagent was used in phosphate flotation on a different sample of ore from that referred to in Example 2. A flotation of the same phosphate ore was also conducted with the reagent referred to in Example 2 and with technical tallow amine acetate. The results obtained are indicated in the following table:

20 containing from 1-4 carbon atoms, and a small proportion of a cationic dispersant.

3. A fluid amine product comprising from 80 to 90% of a long chain fatty amine containing from 14-22 carbon atoms and from 10 to 20% of an ether alcohol having the formula  $ROC_2H_4OH$  in which R is an alkyl group containing from 1-4 carbon atoms, and a small proportion of a salt of the amine with a water soluble acid.

4. A fluid amine product comprising from 80 to 90% of tallow amine and from 10 to 20% of 2-ethoxyethanol and from .1 to 1% of acetic acid based on the weight of the tallow amine.

5. A fluid amine comprising from 80 to 85% of tallow amine, from 15 to 20% of 2-ethoxyethanol and sufficient acetic acid to form a salt of from 2 to 3% of the amine.

35

| Run    | Reagent                                                       | lbs.<br>Reagent<br>per ton | Phosphate Concentrate |                |              |                          | Silica Tailing |                |              | Percent<br>BPL<br>Recovery |
|--------|---------------------------------------------------------------|----------------------------|-----------------------|----------------|--------------|--------------------------|----------------|----------------|--------------|----------------------------|
|        |                                                               |                            | Percent<br>Wt.        | Percent<br>BPL | BPL<br>Units | Percent<br>HCl<br>Insol. | Percent<br>Wt. | Percent<br>BPL | BPL<br>Units |                            |
| 1..... | 80% Tech. Tallow Amine, 19½% 2-ethoxyethanol, ½% Acetic Acid. | 0.35                       | 86.0                  | 85.8           | 73.8         | 3.67                     | 14.0           | 16.7           | 2.3          | 97.0                       |
| 2..... | 85% Tech. Tallow Amine, 14½% 2-ethoxyethanol, ½% Acetic Acid. | 0.32                       | 84.9                  | 85.1           | 72.3         | 3.54                     | 15.1           | 21.5           | 3.2          | 95.8                       |
| 3..... | Tech. Tallow amine acetate.....                               | 0.36                       | 81.0                  | 78.9           | 63.9         | 2.19                     | 19.0           | 27.3           | 5.2          | 92.5                       |

The above table shows that the results obtainable in runs 1 and 2 are nearly identical although less reagent was used in run No. 2. While run No. 3 demonstrated a better grade of concentrate (2.19% insolubles) it sacrificed recovery by from 3 to 5 units. In view of the above it is preferred to employ approximately 85% of the fatty amine in the reagent, but this may be varied from 80 to 90%.

Now, therefore, we claim:

1. A fluid amine product comprising from 80 to 90% of a long chain fatty amine containing from 14-22 carbon atoms and from 10 to 20% of an ether alcohol having the formula  $ROC_2H_4OH$  in which R is an alkyl group containing from 1-4 carbon atoms, and a small proportion of a dispersant selected from the group consisting of cationic and non-ionic dispersants.

2. A fluid amine product comprising from 80 to 90% 65

**References Cited in the file of this patent**

**UNITED STATES PATENTS**

- 2,298,281 Corley et al. ----- Oct. 13, 1942  
2,307,397 Falconer et al. ----- Jan. 5, 1943  
2,377,129 Christmann et al. ----- May 29, 1945  
2,551,197 Barr ----- May 1, 1951  
2,724,501 Hollingsworth et al. ----- Nov. 22, 1955

**FOREIGN PATENTS**

- 993,892 France ----- Aug. 3, 1951

**OTHER REFERENCES**

"Synthetic Organic Chemicals," twelfth edition (1945), pub. by Carbide and Carbon Chemicals Corporation of New York, N. Y., page 37.

"Armeens," pamphlet pub. by Armour Chemical Div. of Armour and Company, Chicago, Illinois (August 1949), pages 5 and 6.